

# United States Patent

[19]

Courcier et al.

[11] 3,816,309

[45] June 11, 1974

[54] **FRICITION MATERIAL**

[75] Inventors: **Francois Courcier, Mun Saint-Maur; Jean Blouet; Robert Courtel**, both of Paris; **Rene Gras, Eaubonne**, all of France; **Francis Risler, Universite de Shubrooke Quebec, Canada**

[73] Assignee: **Commissariat a l'Energie Atomique, Paris, France**

[22] Filed: **July 13, 1971**

[21] Appl. No.: **162,215**

**Related U.S. Application Data**

[63] Continuation-in-part of Ser. No. 829,248, June 2, 1969, abandoned.

[30] **Foreign Application Priority Data**

June 27, 1968 France..... 68.15677Z

[52] U.S. Cl. .... 252/12

[51] Int. Cl. .... C10m 7/02

[58] Field of Search ..... 252/12, 12.2, 12.4, 12.6

[56]

**References Cited**

**UNITED STATES PATENTS**

|           |        |                    |        |
|-----------|--------|--------------------|--------|
| 3,573,204 | 3/1971 | Van Wyk.....       | 252/12 |
| 3,652,408 | 3/1972 | Korshak et al..... | 252/12 |

*Primary Examiner*—Daniel E. Wyman

*Assistant Examiner*—I. Vaughn

*Attorney, Agent, or Firm*—Cameron, Kerkam, Sutton, Stowell & Stowell

[57]

**ABSTRACT**

The friction material consists of a mixture of chromic oxide and 5 to 25 of zirconium oxide. At least a third oxide such as neodymium oxide may be added to the mixture and known lubricants such as graphite, molybdenum bisulfide, calcium or barium fluoride may also be added to the mixture.

**1 Claim, 1 Drawing Figure**

PATENTED JUN 11 1974

3,816,309



1  
FRICTION MATERIAL

## REFERENCE TO RELATED APPLICATION

This application is a continuation-in-part of our application Ser. No. 829,248, filed June 2, 1969, for Friction Material, which application is abandoned.

The present invention relates to a novel friction material, especially for dry friction, which is more especially adapted to constitute a surface coating for parts in relative motion.

It is known that some particular environments such as high-temperature media, nuclear media, corrosive atmospheres, high vacua and the like can call for the use of appliances or mechanisms constructed by means of parts formed of special materials. It is also known that the atmospheres in which such appliances are caused to operate do not permit the use of conventional lubricants in the majority of cases.

The present invention is directed to a novel material which meets the above-mentioned requirements and permits dry friction of moving parts with appreciable reduction of wear of these latter and a substantial reduction of the dangers of seizure.

To this end, said material is characterized in that it

part or in the form of a coating. In the first case, any powder metallurgy technique may be adopted for the formation of such solid parts. In the second case, recourse may be had to techniques such as oxide coating or metallic coating followed by application of oxides. In particular, it is of interest to employ ordinary flame-spray processes or plasma-spray processes. The spray gun can be fed with material in either powder or rod form, the oxides being first mixed together or sprayed at the same time. The plasma-spray gun (jet) can be fed with oxides either in the pure or mixed state. In particular, it is thus possible to apply a thin coating of the oxide mixture to the part to be coated by spraying with the plasma jet a fine powder having a particle size between 10 and 40 microns at a rate of 50 l/min. of argon and a power of 21 kW (700 amps 30 volts).

The table given below by way of indication summarizes a number of tests carried out on parts and especially on a journal mounted in a journal-bearing, the material which constitutes said parts being provided or not provided with a surface coating in accordance with the invention. Results of tests carried out under the following conditions: Dry friction, load of 30 decanewtons, linear speed 0.14 m/sec.

| Nature of journal material                                     | Nature of bearing material     | Coeffi-<br>cient of<br>friction | Duration of<br>test in hours | Total weight loss<br>during testing of— |                      | Remarks                     |
|----------------------------------------------------------------|--------------------------------|---------------------------------|------------------------------|-----------------------------------------|----------------------|-----------------------------|
|                                                                |                                |                                 |                              | Journal,<br>in grams                    | Bearing,<br>in grams |                             |
| Stainless steel                                                | Stainless steel                | 0.9                             | 0 hr. 32 mins.               | 1.45                                    | 0.13                 | Violent seizure.            |
| Chrome stainless steel                                         | Chrome stainless steel         | 0.85                            | 0 hr. 45 mins.               | 1.52                                    | 0.011                | Very rapid wear of journal. |
| Cr <sub>2</sub> O <sub>3</sub>                                 | Cr <sub>2</sub> O <sub>3</sub> | 0.3                             | 46 hrs.                      | 0.06                                    | 0.07                 | Rapid wear and seizure.     |
| ZrO <sub>2</sub>                                               | ZrO <sub>2</sub>               | 1                               | 0 hr. 1 min.                 | 0.30                                    | 0.07                 | Seizure.                    |
| Mixture Cr <sub>2</sub> O <sub>3</sub> -ZrO <sub>2</sub> (15%) | Cr <sub>2</sub> O <sub>3</sub> | 0.25                            | 400 hrs.                     | 0.04                                    | 0.04                 | Very low wear.              |

is made up of a mixture of chromic oxide and zirconium oxide in variable proportions. Preferably, the per-

In addition, the following results have been obtained on a frictiograph at high temperature under vacuum:

| Pair of materials                                | Load        | Speed,<br>m./sec. | Atmosphere                         | Duration<br>of test | Coeff.<br>of<br>fric-<br>tion | Remarks                                           |
|--------------------------------------------------|-------------|-------------------|------------------------------------|---------------------|-------------------------------|---------------------------------------------------|
| Cr <sub>2</sub> O <sub>3</sub>                   | 500 Newtons | 0.14              | 3×10 <sup>-3</sup> torr at 500° C. | 1 hr.               | 0.8                           | Very stable coefficient. Little wear. No seizure. |
| ZrO <sub>2</sub> /Cr <sub>2</sub> O <sub>3</sub> |             |                   |                                    |                     |                               |                                                   |

centage of zirconium oxide in the initial mixture is comprised between 5 and 25 percent.

A reduction in the weight percentage of the zirconium oxide leads to an increase in wear and in the coefficient of friction. Similarly, an excessive increase in the weight percentage of zirconium oxide also gives rise to the same disadvantages. However, within the weight limits mentioned above, experience has shown that a greater degree of stability and regularity of the coefficient of friction are obtained with the highest percentages of zirconium oxide. This material very readily permits incorporation of additives which have known lubricating properties such as graphite, molybdenum bisulphide, calcium fluoride or barium fluoride which are subsequently incorporated in the material. Moreover, it has been observed experimentally that an improvement in the qualities of the friction material could be achieved by adding at least a third oxide to the mixture of chromic oxide and zirconium oxide. Advantageously, this third oxide is neodymium oxide.

The friction material under consideration can be utilized in two forms, namely either in the form of a solid

By way of explanatory illustration, the single FIGURE of the accompanying drawings relates to tests on continuous coatings of mixtures of chromic oxide with zirconium oxide in variable proportions. The curves which are plotted relate to wear and to the coefficient of friction in ambient air of a journal formed of nitrided steel and coated with a mixture of chromic oxide and zirconia having a thickness of 2/10 mm on a bearing-block formed of the same steel and coated with pure chromic oxide.

The parts are placed in contact with each other and loaded prior to setting the machine in operation. The machine is stopped 3 hours after start-up. The journal and the bearing remain in contact and under load for a period of 1 hour. At the end of this period, the machine is again started up for a further cycle which lasts 4½ hours.

1. Friction material consisting essentially of a mixture of chromic oxide and zirconium oxide the percentage of zirconium oxide in the mixture of chromic oxide and zirconium oxide being from about 5 to about 25 percent.